

## UNITED STATES PATENT OFFICE

2,133,847

## CORROSION RESISTANT TUBULAR ARTICLE

Donald K. Crampton, Marion, and Newell W. Mitchell, Waterbury, Conn., assignors to Chase Brass & Copper Co., Incorporated, Waterbury, Conn., a corporation of Connecticut

No Drawing. Application March 30, 1936,  
Serial No. 71,808

6 Claims. (Cl. 138—47)

This invention relates to improvements in corrosion-resistant tubular articles, and more particularly, corrosive-resistant wrought-metal tubular articles formed of copper-base alloys containing phosphorus, aluminum, zinc and tin, with or without other elements which do not seriously impair the properties of the alloy.

We have found that wrought-metal tubular articles, such, for example, as tubes, pipes, etc., made of copper-base alloys containing phosphorus from about  $\frac{1}{4}\%$  to about 2%, aluminum from about  $\frac{1}{4}\%$  to about 4%, zinc from about 1% to about 30%, tin from about  $\frac{1}{2}\%$  to about 3 $\frac{1}{2}\%$ , and copper, the copper, phosphorus, aluminum, zinc and tin constituting about 90% or more of the alloy, with or without one or more additional elements in such substantially-innocuous amounts as do not seriously impair the properties of the alloy, have valuable corrosion-resistant properties, especially when in contact with saline liquid or dilute acid. The additional elements may range up to a total of about 10%, depending on what elements are added, some being more innocuous than others.

While each of the elements iron, antimony and arsenic should not be present much in excess of about 0.1%, silver, which is comparatively innocuous may be present to as high as about 10% provided not too much of other elements is present. Nickel may be present to as high as about 5%, lead may be present to as high as about 3 $\frac{1}{2}\%$ , silicon may be present to as high as about 3%, and manganese may be present to as high as about 1%.

The phosphorus may range from about  $\frac{1}{4}\%$  to about 2%, the aluminum from about  $\frac{1}{4}\%$  to about 4%, the zinc from about 1% to about 30% and the tin from about  $\frac{1}{2}\%$  to about 3 $\frac{1}{2}\%$ , and the zinc preferably should be in such quantity, not more than about 30%, as to have the alloy consist entirely of the alpha phase, with the sum of the phosphorus, aluminum and tin contents 6 or less for zinc contents of 20% or more and 7 or less for zinc contents of less than 20%.

It is still more preferable to have the phosphorus from about  $\frac{1}{2}\%$  to about 1 $\frac{1}{2}\%$ , the aluminum from about 1% to about 3%, the zinc from about 5% to about 20%, and the tin from about 1% to about 3%, and preferably the sum of the phosphorus, aluminum and tin contents should be 6 or less.

It is even more preferable to have the phosphorus from about  $\frac{1}{2}\%$  to about 1%, the aluminum from about 1% to about 2%, the zinc from

about 5% to about 15%, and the tin from about 1% to about 3%. And within this range three alloys may be advantageously made having nominal composition as follows: all three have about 1 $\frac{1}{2}\%$  aluminum and about 10% zinc, the first having about 1% phosphorus and about 3% tin, the second having about 3 $\frac{1}{4}\%$  phosphorus and about 2% tin, and the third having about  $\frac{1}{2}\%$  phosphorus and about 2 $\frac{1}{2}\%$  tin.

The invention may be carried out in other specific ways than those herein set forth without departing from the spirit and essential characteristics of the invention, and the present embodiments are therefore to be considered in all respects as illustrative and not restrictive, and all changes coming within the meaning and equivalency range of the appended claims are intended to be embraced therein.

We claim:

1. A wrought-metal tubular article for use in contact with saline liquid or dilute acid and characterized by good corrosion resistance to saline liquid and dilute acid and formed from an alloy containing: phosphorous as an essential element from about  $\frac{1}{4}\%$  to about 2%; aluminum from about  $\frac{1}{4}\%$  to about 4%; zinc from about 1% to about 30% and in such quantity as to have the alloy consist entirely of the alpha phase with the sum of the phosphorus, aluminum and tin 6 or less when the zinc is 20% or more, and 7 or less when the zinc is less than 20%; tin from about  $\frac{1}{2}\%$  to about 3 $\frac{1}{2}\%$ ; and the balance substantially of copper.

2. A wrought-metal tubular article for use in contact with saline liquid or dilute acid and characterized by good corrosion resistance to saline liquid and dilute acid and formed from an alloy containing: phosphorus as an essential element from about  $\frac{1}{2}\%$  to about 1 $\frac{1}{2}\%$ ; aluminum from about 1% to about 3%; zinc from about 5% to about 20%; tin from about 1% to about 3%; and the balance substantially of copper.

3. A wrought-metal tubular article for use in contact with saline liquid or dilute acid and characterized by good corrosion resistance to saline liquid and dilute acid and formed from an alloy containing: phosphorus as an essential element from about  $\frac{1}{2}\%$  to about 1%; aluminum from about 1% to about 2%; zinc from about 5% to about 20%; tin from about 1% to about 3%; and the balance substantially of copper.

4. A wrought-metal article for use in contact with saline liquid or dilute acid and characterized by good corrosion resistance to saline liquid and dilute acid and formed from an alloy containing:

- phosphorus as an essential element about 1%; aluminum about 1½%; zinc about 10%; tin about 3%; and the balance substantially of copper.
5. A wrought-metal tubular article for use in contact with saline liquid or dilute acid and characterized by good corrosion resistance to saline liquid and dilute acid and formed from an alloy containing: phosphorus as an essential element about ½%; aluminum about 1½%; zinc about 10%; tin about 2½%; and the balance substantially of copper.
10. A wrought-metal tubular article for use in contact with saline liquid or dilute acid and characterized by good corrosion resistance to saline liquid and dilute acid and formed from an alloy containing: phosphorus as an essential element about ¾%; aluminum about 1½%; zinc about 10%; tin about 2%; and the balance substantially of copper.
6. A wrought-metal tubular article for use in contact with saline liquid or dilute acid and characterized by good corrosion resistance to saline liquid and dilute acid and formed from an alloy containing: phosphorus as an essential element about ½%; aluminum about 1½%; zinc about 10%; tin about 2½%; and the balance substantially of copper.

5

DONALD K. CRAMPTON. 10  
NEWELL W. MITCHELL.